

Feb. 4, 1958

E. F. KURZINSKI

2,821,760

FLAME HEATING OF METAL CASTINGS TO REDUCE SHRINKAGE CAVITIES

Filed Dec. 24, 1956

*Fig. 1.*



*Fig. 2.*



*Fig. 3.*



*Fig. 4.*



INVENTOR  
EDWARD F. KURZINSKI  
BY  
*D. Harrision*  
ATTORNEY

1

2,821,760

## FLAME HEATING OF METAL CASTINGS TO REDUCE SHRINKAGE CAVITIES

Edward F. Kurzinski, Cranford, N. J., assignor to Union Carbide Corporation, a corporation of New York

Application December 24, 1956, Serial No. 630,419

3. Claims. (Cl. 22—216)

This invention relates to a novel process for heating a freshly poured casting of molten metal to eliminate or reduce the size of the shrinkage cavity which normally forms near the top of a casting during solidification.

The application of heat to the top portion of a metal casting such as an ingot hot-top or a casting riser for reducing shrinkage cavities has been known for many years, both electrical and gas heating having been suggested. However, prior to the present invention a number of disadvantages have prevented gas heating from being employed on a commercial scale.

One of the principal disadvantages of gas heating was the need for water-cooling the gas burner to protect it from destruction by the heat of the operation. In a foundry or steel mill where molten metals such as steel are being cast from ladles into molds, the water-cooling of a burner is undesirable for several reasons. If a leak occurs in the water-cooling system a dangerous situation can be created by the discharge of leaking water against the molten metal, and the hot refractories which are employed. Water-cooling also creates an undesirable complication of equipment because two additional conduits for water must be used. Moreover, in cold weather water in the conduits may freeze when the apparatus is out of use.

In accordance with the present invention there is provided a process for producing a solid metal casting which is substantially free from a shrinkage cavity by pouring the molten metal into a mold to form a casting, positioning a gas burner nozzle above the top surface of the casting, and applying from the nozzle against the top surface an oxy-fuel gas flame of the blow-off type to keep the top of the casting molten while the rest of the metal solidifies. A blow-off type of flame is produced when the oxy-fuel gas mixture starts to burn at a point spaced from the face of the burner nozzle, rather than right at the face as with conventional flames.

The blow-off oxy-fuel gas flame used in my process is formed by so correlating the ratio of oxygen to fuel gas in the combustible mixture with the discharge velocity of the mixture that the flame starts to burn at a point spaced off the face of the burner nozzle. Its combustion sometimes must be maintained by the igniting effect of some additional heating agency, such as the heat of the incandescent metal casting itself. For example, when the gas velocity is 500 feet per second the flame will not burn in the free atmosphere, but requires the igniting effect of a hot body to keep it burning. The point at which the flame starts to burn varies dependent upon the velocity of the combustible mixture and the distance between the nozzle and the top of the metal casting. In some instances the flame has been spaced as little as one-eighth inch from the nozzle face; and in others one-half inch spacing has occurred.

When a blow-off flame is employed in the manner described in the preceding paragraph, the burner is subjected principally to the heat emanating from the metal casting and is heated only slightly by the flame itself, much less than in the case of a conventional oxy-fuel gas flame

2

burning at the face of the nozzle. Consequently it has been found feasible to employ a burner without a water-cooling system when using a blow-off flame.

To produce the blow-off type of flame which is employed in my novel process, the oxy-fuel gas mixture should flow at a calculated discharge velocity (quantity of gas flowing/total area of orifice) greater than 200 feet per second as it leaves the burner nozzle, and the ratio of oxygen to fuel gas in the mixture should be maintained between 1.3 and 1.8 to 1. A discharge velocity of about 500 feet per second has been found advantageous. Velocities in excess of 1000 feet per second are not desirable.

By using the process described above it has been found possible to reduce the volume of metal required in the hot-top from 15% down to 7% of the ingot volume while maintaining the main body of the ingot sound and free from shrinkage cavities.

Specific ways of employing the principles of the invention will be described in detail below with reference to the accompanying drawing, wherein:

Fig. 1 is a perspective view showing an ingot mold filled with molten steel being treated by the process of the invention;

Fig. 2 is an enlarged vertical sectional view of the mold and part of the burner shown in Fig. 1;

Fig. 3 is an elevational view of the burner as seen from below in Fig. 2; and

Fig. 4 is a perspective view, partially broken away and shown in section, of another type of casting being treated by the process of the invention.

As shown in Fig. 1 an ingot mold 11 carrying a conventional ceramic hot-top 13 having an integral annular cover 14 provided with an aperture 16 has been filled with molten steel 15 to a level within the hot-top.

After filling the mold a burner 19 has been placed in position with its burner nozzle 21 above the aperture 16 and the top surface of the casting 15. Immediately after positioning the burner 19 above the casting, a fuel gas such as natural gas (which is predominantly methane) is supplied to a gas mixer body 23 through a supply conduit 25 which is provided with an adjustable automatic pressure regulator 27. Simultaneously the flow of oxygen is commenced to the mixer body 23 through a supply conduit 29 having therein an adjustable automatic pressure regulator 31. The two gases mix intimately together within the body 23 and the resulting combustible mixture passes through the burner to the nozzle 21 from which it is discharged through a plurality of ports 33 against the casting 15. The mixer body 23 may include any conventional mixer construction, as is well known in blowpipes, for example as shown and described in United States Patent 2,242,471.

The proper ratio of the oxygen to fuel gas in the combustible mixture is determined by adjusting the settings of the pressure regulators 27 and 31. The proper velocity of the discharged combustible mixture is assured by providing the burner nozzle 21 with noncounterbored drilled ports 33 such that their aggregate cross-sectional area produces the desired velocity for a given quantity flow of mixture through the burner 19, as is well known to those skilled in the art.

The elimination of water-cooling and the employment of blow-off flames have made it possible to employ a burner 19 of an extremely simple and inexpensive construction. The burner shown only requires a length of iron pipe 35, the street L 37 threaded over the front end of the pipe, and a pipe cap 39 threaded over the end of the street L and having the discharge orifices 33 drilled therein.

The number, arrangement, and inclination of the dis-

charge orifices 33 can be varied as desired to suit the type of casting being treated, within the scope of the invention. The particular nozzle shown in Figs. 1 and 2 is provided with four orifices arranged as the corners of a square and having their axes diverging downwardly and outwardly from one another so as to direct the flames toward the periphery of the casting 15.

Partially covering the top of the casting 15, as by the annular cover 14, reduces gas consumption considerably over the amount consumed when no cover is used, the saving in gas being as much as 50% in some instances.

In a modified form of apparatus, as shown in Fig. 4, a long and narrow casting 41 is treated with two groups of blow-off flames 43 and 45 projected simultaneously from a pair of nozzles 47 and 49 connected to a single pipe 51 which is supplied with a combustible mixture from a mixer body (not shown) similar to the mixer body 23 shown in Fig. 1.

Several specific examples of how the process of the invention has been successfully carried out for treating metal castings are described in detail below as an aid to persons skilled in the art who may wish to practice the invention.

In all examples the top of the ingot was flat and no shrinkage cavities extended down into the main body of the ingot. Also, the burner was in reusable condition after conclusion of the treatment.

#### Example 1

A partially covered ingot of stainless steel weighing 3 tons and having a rectangular top 15 x 28 inches and having a hot-top containing 5 inches depth of metal, in contrast to the conventional 8 inches, was treated with a blow-off flame for 1 hour while holding a non-water-cooled burner nozzle 4 inches from the surface of the metal. The blow-off flame was formed by discharging from the burner nozzle at 500 feet per second a 1.53:1 ratio combustible mixture formed from oxygen and natural gas flowing at 827 and 540 cubic feet per hour, respectively.

#### Example 2

A partially covered ingot of nickel-molybdenum tool steel weighing 4500 pounds and having a cylindrical top 19 inches in diameter was provided with a hot-top one-half the depth normally used on such ingots. The ingot then was treated with a blow-off flame for 1 hour while holding a non-water-cooled burner nozzle 8½ inches from the surface of the metal. The blow-off flame was formed by discharging from the burner nozzle at 500 feet per second a 1.52:1 ratio combustible mixture formed from oxygen and natural gas flowing at 500 and 333 cubic feet per hour, respectively.

#### Example 3

A partially covered ingot of carbon steel weighing 9000 pounds and having a rectangular top 22 x 25 inches was treated with blow-off flames from two nozzles for 65 minutes while holding the two non-water-cooled nozzles 12 inches from the surface of the metal in the hot-top. The blow-off flames were formed by discharging from both burner nozzles at 500 feet per second a 1.8:1 ratio combustible mixture formed from oxygen and natural gas flowing at 975 and 540 cubic feet per hour, respectively.

The overall yield of usable steel was 85%, in contrast to 76% obtained without treatment.

#### Example 4

A partially covered ingot of chromium-molybdenum-vanadium tool steel was poured with a hot-top constituting 7½% of the ingot volume, in contrast to 15% in normal practice. The casting then was treated with a cluster of blow-off flames for 14 minutes from a burner nozzle positioned 4 inches above the metal surface. The flame was formed by burning a combustible mixture flow-

ing at 300 feet per second, and formed from 300 cubic feet per hour of oxygen and 200 cubic feet per hour of natural gas (a 1.5:1 ratio).

#### Example 5

An ingot of stainless steel weighing 7360 pounds and having a rectangular top 16 x 31 inches was treated with a blow-off flame for 50 minutes from a burner nozzle positioned 2½ inches above the metal surface while leaving the hot-top uncovered. The hot-top had been filled with 390 pounds less metal than usual. The flame was formed by burning a combustible mixture flowing at 500 feet per second, and formed from 1194 and 667 cubic feet per hour, respectively, of oxygen and fuel gas.

15

#### Example 6

An ingot of stainless steel weighing 6340 pounds and having a rectangular top 15 x 28 inches was poured with an uncovered hot-top and the surface of the metal

20

was covered with silica. A blow-off flame was then applied to the top of the casting for 50 minutes from a burner nozzle located 3½ inches above the top. Oxygen and fuel gas were supplied at 923 and 660 cubic feet per hour, respectively, and the mixture flowed at a

25

velocity of 500 feet per second.

Only 4.1% of the ingot volume contained a pipe, in contrast to the 9% normal pipe.

This application is in part a continuation of my co-pending application Serial No. 265,942, filed January 11,

30

1952, now abandoned, and combines therewith the use of slags in combination with the blow-off flame for hot-topping, and the oxy-fuel ratios for the use of propane and coke-oven gas and city gas for fuel.

35

The slags can be naturally-occurring materials such as wollastonite or specially prepared synthetics such as disclosed in Jones et al. Patent No. 2,043,960.

#### Examples

|                                              | I    | II    | III   | IV    |
|----------------------------------------------|------|-------|-------|-------|
| 40                                           |      |       |       |       |
| Percent CaO.....                             | 29.5 | 31.24 | 29.18 | 40.12 |
| Percent MgO.....                             | 8.7  | 11.01 | 8.26  | 0.89  |
| Percent SiO <sub>2</sub> .....               | 56.4 | 52.40 | 57.48 | 52.94 |
| Percent Al <sub>2</sub> O <sub>3</sub> ..... | 5.4  | 4.11  | 4.86  | 5.80  |
| Percent Fe <sub>2</sub> O <sub>3</sub> ..... | Low  | 0.13  | 0.24  | 0.23  |

45

The advantages of using slags are: They eliminate depletion of readily oxidizable elements in the steel. They permit heating with higher oxy-fuel gas ratios and thereby take advantage of higher flame temperatures. They permit successful hot-topping of large size ingots.

50

In treating small size ingots, up to about 15-in. square and depending upon metal chemistry, the primary purpose of the slag is to prevent oxidation of elements which may cause porosity in the hot-top—the major element being carbon. Many alloy steels can be hot-topped using oxy-fuel gas flames in these smaller ingot sizes without requiring slags as barriers.

55

In hot-topping large size ingots, the problem is completely different. Solidification of ingots is expressed as:

$$T = K \left( \frac{d}{2} \right)^2$$

Where:

60  $T$ =Ingot solidification time (min.)  
 $K$ =Co-efficient dependent upon ingot mold characteristics and heating time  
 $d$ =Smallest dimension of ingot (in.)

Using this formula and for simplicity assuming  $K=1$ , the solidification time for a 10-in. square ingot will be 25 min., whereas, this increases to 225 min. for a 30-in. ingot. Large size ingots are exposed, therefore, to the oxidizing influence of the oxy-fuel gas combustion products for a proportionally longer period. Thus, where oxidation would not be a factor on small size ingots of

a specific metal chemistry, the problem becomes increasingly difficult as ingot size increases. For example, 10 x 10 in. ingots of type 304 stainless can easily be heated using oxy-natural gas ratios of 1.5:1. In heating large size ingots, 22 x 25 in., the oxy-natural gas ratio would have to be reduced to 1.1:1 to overcome the effect of oxidation by the combustion products. Using this ratio, there is insufficient heat in the combustion products to effectively hot-top the ingot. The difficulty is caused by the appearance of a powdery slag being formed on the surface of the metal in the hot-top as the heating progresses. This powdery slag probably contains considerable amounts of chromium oxide which is highly refractory. The refractory character of this slag causes considerable heat reflection which substantially decreases the amount of heat made available to the metal in the hot-top. On type 321 stainless, an equally unsatisfactory condition is experienced; however, this slag has a slushy character.

Initial experiments were made introducing crushed glass on the surface of the hot-top prior to the start of heating. This is satisfactory in most cases. Synthetic slags such as those according to Patent No. 2,043,960 are more desirable than crushed glass in instances because of more uniform slag chemistry, control of viscosity, better sizing and ready availability. The disadvantage of synthetic slags is that the cost is higher.

In treating ingots under production conditions, it is desirable in some cases to add exothermic materials to the synthetic slags. The exothermic material imparts heat to the hot-top surface to retard solidification until the teeming ladle is moved sufficiently for the heating tips to be positioned over the ingots.

Timing between the slag addition and the start of heating is important. In treating a 9 x 9 in. ingot, 20 x 200 slag according to Patent No. 2,150,625

#### Examples

|                                              | I    | II    | III   | IV    |
|----------------------------------------------|------|-------|-------|-------|
| Percent CaO.....                             | 29.5 | 31.24 | 29.18 | 40.12 |
| Percent MgO.....                             | 8.7  | 11.01 | 8.26  | 0.89  |
| Percent SiO <sub>2</sub> .....               | 56.4 | 52.40 | 57.48 | 52.94 |
| Percent Al <sub>2</sub> O <sub>3</sub> ..... | 5.4  | 4.11  | 4.86  | 5.80  |
| Percent Fe <sub>2</sub> O <sub>3</sub> ..... | Low  | 0.13  | 0.24  | 0.23  |

and 40% periclase, was placed on the surface of the hot-top and the heating flames started immediately thereafter. The high velocity of the blow-off flames ejected the slag material out of the hot-top. A short delay period is desirable from the time of slag addition to turning on the heating flames to permit the slags to partially fuse. On many grades of high-speed and tool steels, 1 in. XD wollastonite was effective in preventing oxidation of elements in the steel.

Two examples are given to illustrate the effectiveness of slags in heating large size ingots:

#### Example 7

15 x 28 in., 6350 lb. ingot of type 430 stainless was heating using 928 cu. ft. per hour oxygen and 660 cu. ft. per hour of natural gas and the blowoff flame technique. The heating time was 50 minutes. Using slags, the top crop was 4.1 percent while for conventional practice ingots, the top crop was 10 percent. Oxy-natural gas hot-topping would not have been possible using this ratio on this ingot size without the use of slag.

#### Example 8

22 x 25 in., 7000 lb. ingot of type 304 stainless steel 70 was heating using 1640 cu. ft. per hour of oxygen, 480 cu. ft. per hour of propane, glass slag and blowoff flame. Ingot yield was 88 percent including top crop, bottom crop and scale loss. The regular cast ingot made for comparative purposes showed a yield of 80 percent. 75

Again, this ingot could not have been hot-topped without the use of the slag.

When using propane, coke-oven and city gas, the ranges of the oxy-fuel gas ratios are:

|   |                                  |                |
|---|----------------------------------|----------------|
| 5 | Oxy-Propane .....                | 2.5:1 to 4.0:1 |
|   | Oxy-Coke oven and city gas ..... | 0.5:1 to 1.1:1 |

What is claimed is:

1. In the process of treating a freshly poured molten metal casting to keep the top of the casting molten while said casting solidifies from the bottom to the top thereof to reduce the size of the shrinkage cavity therein, wherein an oxy-fuel flame is directed against the top surface of said casting during such cooling, the improvement which comprises in combination therewith positioning a burner nozzle above the top surface of said casting and vertically spaced therefrom a distance such that overheating of the nozzle is avoided, and applying from said burner nozzle against said top surface an oxy-fuel gas mixture having an oxygen to fuel gas ratio of from 1.3:1 to 1.8:1 and a velocity of from 200 feet per second to 1000 feet per second, to burn said mixture with a stable blow-off flame by continuous ignition thereof by the molten casting.
2. In the process of treating a freshly poured molten metal casting to keep the top of the casting molten while said casting solidifies from the bottom to the top thereof to reduce the size of the shrinkage cavity therein, wherein an oxy-fuel flame is directed against the top surface of said casting during such cooling, the improvement which comprises in combination therewith positioning a burner nozzle above the top surface of said casting and vertically spaced therefrom a distance such that overheating of the nozzle is avoided, and applying from said burner nozzle against said top surface an oxy-fuel gas mixture having an oxygen-to-fuel gas ratio of from 1.3:1 to 1.8:1 for natural gas, 2.5:1 to 4.0:1 for propane and 0.5:1 to 1.1:1 for coke oven and city gas and a velocity of from 200 feet per second to 1000 feet per second, to burn said mixture with a stable blow-off flame by continuous ignition thereof by the molten casting.
3. In the process of treating a freshly poured molten metal casting to keep the top of the casting molten while said casting solidifies from the bottom to the top thereof to reduce the size of the shrinkage cavity therein, wherein an oxy-fuel flame is directed against the top surface of said casting during such cooling, the improvement which comprises in combination therewith introducing slag on the surface of the hot-top to overcome the effect of oxidation by the combustion products and prevent reflection by refractory oxides, positioning a burner nozzle above the top surface of said casting and vertically spaced therefrom a distance such that overheating of the nozzle is avoided, and applying from said burner nozzle against said top surface an oxy-fuel gas mixture having an oxygen-to-fuel gas ratio of from 1.3:1 to 1.8:1 for natural gas, 2.5:1 to 4.0:1 for propane and 0.5:1 to 1.1:1 for coke oven and city gas and a velocity of from 200 feet per second to 1000 feet per second, to burn said mixture with a stable blow-off flame by continuous ignition thereof by the molten casting.

4. In the process of treating a freshly poured molten metal casting to keep the top of the casting molten while said casting solidifies from the bottom to the top thereof to reduce the size of the shrinkage cavity therein, wherein an oxy-fuel flame is directed against the top surface of said casting during such cooling, the improvement which comprises in combination therewith positioning a burner nozzle above the top surface of said casting and vertically spaced therefrom a distance such that overheating of the nozzle is avoided, and applying from said burner nozzle against said top surface an oxy-fuel gas mixture having an oxygen-to-fuel gas ratio of from 1.3:1 to 1.8:1 for natural gas, 2.5:1 to 4.0:1 for propane and 0.5:1 to 1.1:1 for coke oven and city gas and a velocity of from 200 feet per second to 1000 feet per second, to burn said mixture with a stable blow-off flame by continuous ignition thereof by the molten casting.
5. In the process of treating a freshly poured molten metal casting to keep the top of the casting molten while said casting solidifies from the bottom to the top thereof to reduce the size of the shrinkage cavity therein, wherein an oxy-fuel flame is directed against the top surface of said casting during such cooling, the improvement which comprises in combination therewith positioning a burner nozzle above the top surface of said casting and vertically spaced therefrom a distance such that overheating of the nozzle is avoided, and applying from said burner nozzle against said top surface an oxy-fuel gas mixture having an oxygen-to-fuel gas ratio of from 1.3:1 to 1.8:1 for natural gas, 2.5:1 to 4.0:1 for propane and 0.5:1 to 1.1:1 for coke oven and city gas and a velocity of from 200 feet per second to 1000 feet per second, to burn said mixture with a stable blow-off flame by continuous ignition thereof by the molten casting.

#### References Cited in the file of this patent

#### UNITED STATES PATENTS

|    |           |                      |               |
|----|-----------|----------------------|---------------|
| 65 | 359,974   | Irwin .....          | Mar. 22, 1887 |
|    | 1,310,072 | Hadfield .....       | July 15, 1919 |
|    | 1,336,234 | Jamison .....        | Apr. 6, 1920  |
|    | 1,671,253 | Parsons et al. ..... | May 29, 1928  |
|    | 1,763,047 | Hepburn .....        | June 10, 1930 |
|    | 1,874,341 | Osthoff .....        | Aug. 30, 1932 |
|    | 1,986,201 | Huff .....           | Jan. 1, 1935  |
|    | 2,116,096 | Caldwell .....       | May 3, 1938   |
|    | 2,116,671 | Trofimov .....       | July 18, 1939 |
|    | 2,353,657 | Edwards et al. ..... | July 18, 1944 |
|    | 2,638,159 | Winkelman .....      | May 12, 1953  |